# EUROPEAN PATENT SPECIFICATION

(11) **EP 0 986 443 B1**
(45) Date of publication and mention of the grant of the patent: **17.12.2003**
(21) Application number: 98923930.6
(22) Date of filing: 02.06.1998
(51) Int. Cl.: B22D 11/06, B22D 11/14, B22D 11/18

(54) **AMORPHOUS OR GLASSY ALLOY SURFACED ROLLS FOR THE CONTINUOUS CASTING OF METAL STRIP**
ROLLEN MIT AMORPHER ODER GLASIGER LEGIERUNGSOBERFLÄCHE ZUM KONTINUIERLICHEN GIESSEN VON METALLBÄNDERN
CYLINDRES REVETUS EN SURFACE D'UN ALLIAGE AMORPHE OU NON CRISTALLIN POUR LA COULEE CONTINUE DE BANDE METALLIQUE

(30) Priority: 02.06.1997 AU PO710497
(43) Date of publication of application: 22.03.2000
(73) Proprietor: Castrip, LLC, Charlotte, NC 28211 (US)
(72) Inventor: STREZOV, Lazar, Adamstown, NSW 2289 (AU)
(74) Representative: Lerwill, John
(86) International application number: AU9800412
(87) International publication number: WO98055251

(56) References cited:
- EP-A- 0 732 163
- WO-A-94/12300
- WO-A-95/13889
- DE-A- 3 742 594
- PATENT ABSTRACTS OF JAPAN vol. 010, no. 044 (M-455), 21 February 1986 (1986-02-21) & JP 60 196209 A (SUMITOMO KINZOKU KOGYO KK), 4 October 1985 (1985-10-04)
- PATENT ABSTRACTS OF JAPAN vol. 011, no. 259 (C-441), 21 August 1987 (1987-08-21) & JP 62 060879 A (NGK INSULATORS LTD;OTHERS: 01), 17 March 1987 (1987-03-17)
- PATENT ABSTRACTS OF JAPAN, CD No. 9, B22, (1976-1993); & JP,A,57 130 750 (NITTETSU HARD KABUSHIKI KAISHA) 13 August 1982.
- PATENT ABSTRACTS OF JAPAN, CD No. 9, B22, (1976-1993); & JP,A,02 160 145 (KAWASAKI STEEL CORPORATION & KOUKA KUROOMU KABUSHIKI KAISHA) 20 June 1990.
- PATENT ABSTRACTS OF JAPAN, CD No. 1997-2(025); & JP,A,08 281 382 (NIPPON STEEL CORPORATION) 29 October 1996.
- PATENT ABSTRACTS OF JAPAN, CD No. 1997-3(026); & JP,A,08 294 751 (NIPPON STEEL CORPORATION) 12 November 1996.

## Description

### TECHNICAL FIELD

This invention relates to the casting of metal strip. It has particular but not exclusive application to the casting of ferrous metal strip.

It is known to cast metal strip by continuous casting in a twin roll caster. In this technique molten metal is introduced between a pair of contra-rotated horizontal casting rolls which are cooled so that metal shells solidify on the moving roll surfaces and are brought together at the nip between them to produce a solidified strip product delivered downwardly from the nip between the rolls. The term "nip" is used herein to refer to the general region at which the rolls are closest together. The molten metal may be poured from a ladle into a smaller vessel or series of vessels from which it flows through a metal delivery nozzle located above the nip so as to direct it into the nip between the rolls, so forming a casting pool of molten metal supported on the casting surfaces of the rolls immediately above the nip and extending along the length of the nip. This casting pool is usually confined between side plates or dams held in sliding engagement with end surfaces of the rolls so as to dam the two ends of the casting pool against outflow, although alternative means such as electromagnetic barriers have also been proposed.

Although twin roll casting has been applied with some success to non-ferrous metals which solidify rapidly on cooling, there have been problems in applying the technique to the casting of ferrous metals. One particular problem has been the achievement of sufficiently rapid and even cooling of metal over the casting surfaces of the rolls.

Our United States Patent 5,520,243 (International Patent Application PCT/AU93/00593) describes a development by which the cooling of metal at the casting surface of the rolls can be dramatically improved by taking steps to ensure that the roll surfaces have certain smoothness characteristics in conjunction with the application of relative vibratory movement between the molten metal of the casting pool and the casting surfaces of the rolls. Specifically that Patent discloses that the application of vibratory movements of selected frequency and amplitude make it possible to achieve a totally new effect in the metal solidification process which dramatically improves the heat transfer from the solidifying molten metal, the improvement being such that the thickness of the metal being cast at a particular casting speed can be very significantly increased or alternatively the speed of casting can be substantially increased for a particular strip thickness. The improved heat transfer is associated with a very significant refinement of the surface structure of the cast metal.

Our United States Patent 5,584,338 describes a further development whereby effective relative vibration between the molten metal of the casting pool and the casting surface can be induced by the application of sound waves to the molten metal of the casting pool whereby increased heat transfer and solidification structure refinement can be achieved by the application of sound waves in the sonic range at quite low power levels.

Our further United States Patent 5,720,336 (corresponding to EP-A-0 732 163) describes the results of research on the heat transfer mechanism occurring at the interface between the casting surface and the molten metal of the casting pool and discloses that the heat flux on solidification can be controlled and enhanced by ensuring that the casting surfaces are each covered by a layer of a material which is at least partially liquid at the solidification temperature of the metal, the liquid of this layer having a wetting angle of less than 40° on the casting surfaces, whereby it is possible to achieve improved heat transfer without necessarily generating relative vibration between the casting pool and the rolls.

In the ensuing description it will be necessary to refer to a quantitative measure of the smoothness of casting surfaces. One specific measure used in our experimental work and helpful in defining the scope of the present invention is the standard measure known as the Arithmetic Mean Roughness Value which is generally indicated by the symbol Rₐ. This value is defined as the arithmetical average value of all absolute distances of the roughness profile from the centre line of the profile within the measuring length lₘ. The centre line of the profile is the line about which roughness is measured and is a line parallel to the general direction of the profile within the limits of the roughness-width cut-off such that sums of the areas contained between it and those parts of the profile which lie on either side of it are equal. The Arithmetic Mean Roughness Value may be defined as

Although the above described developments have enabled the achievement of high solidification rates with the casting of ferrous metal strip it has proved very difficult to produce strip which does not exhibit the surface defect known as "crocodile-skin". This defect occurs when δ and γ iron phases solidify simultaneously in shells on the casting surfaces of the rolls in a twin roll caster under circumstances in which there are variations in heat flux through the solidifying shells. The δ and γ iron phases have differing hot strength characteristics and the heat flux variations then produce localised distortions in the solidifying shells which come together at the nip between the casting rolls and result in the crocodile-skin defects in the surfaces of the resulting strip. Previously this problem has been addressed by endeavouring to keep the build up of oxides on the casting rolls within strict limits by complicated roll cleaning devices.

A light oxide deposit can be beneficial in ensuring a controlled even flux during metal solidification on to the casting roll surfaces. The oxide deposit melts as the roll surfaces enter the molten metal casting pool and assists in establishing a thin liquid interface layer between the casting surface and the molten metal of the casting pool to promote good heat flux. However, if there is too much oxide build up the melting of the oxides produces a very high initial heat flux but the oxides then resolidify with the result the heat flux decreases rapidly. The resulting heat flux variations in the solidifying shells produce the localised distortions leading to crocodile-skin surface defects.

We have now determined that the deleterious effect of the metal oxidation products can be avoided and very high solidification rates can be achieved if the casting surfaces of the rolls are formed of a material which has a high affinity for the molten metal of the casting pools so as to produce extremely good wetting of the casting surface by the molten metal. If there is sufficiently good wetting by the molten metal it is possible for solidification to proceed so rapidly that there is insufficient time for any significant quantities of oxidation products to form. In the case of steel melts it is also possible to achieve rapid solidification of the steel melt into a single phase solid structure thereby effectively avoiding any potential for crocodile-skin defects.

### DISCLOSURES OF THE INVENTION

According to the invention there is provided a method for continuously casting metal strip of the kind in which a casting pool of molten metal is formed in contact with a moving casting surface such that metal solidifies from the pool onto the moving casting surface, wherein the casting surface is provided by a solid coating on a heat conductive body, characterised in that the coating material is so selected that the wetting angle of said molten metal on the coating surface is less than 40°, and the coating material has a melting temperature greater than the temperature of the casting surface during metal solidification.

Preferably further the coating is formed of a material such that the wetting angle of the molten metal on the coating surface is less than 20°.

Preferably the coating surface has an Arithmetic Mean Roughness Value (Rₐ) of less than 10 microns.

The coating material should be chosen so as not to melt or to dissolve in said molten metal at the temperature of the casting surface during solidification.

Preferably, the coating material is at least partially amorphous. It may, for example, comprise an amorphous alloy. One of those components may be phosphorus.

More specifically, the coating material may comprise an amorphous nickel-phosphorus alloy containing about 10% phosphorus.

The heat conductive body may be a body of copper or a copper alloy.

The molten metal may be a ferrous metal.

More specifically, the molten metal may be molten steel. In this case, the choice of a coating material on which the molten steel has a low wetting angle enables solidification of the steel into a single phase solid structure on the casting surface.

Accordingly the invention also provides a method for continuously casting steel strip of the kind in which a casting pool of molten steel is formed in contact with a moving casting surface such that steel solidifies from the casting pool onto the moving casting surfaces, wherein the casting surface is provided by a solid coating on a heat conductive body, characterised that the coating material is so selected that the wetting angle of the molten steel on the coating surface is less than 40°, the temperature of the coating during metal solidification is maintained below the melting temperature of the coating, and wherein the steel solidifies into a single phase solid structure on the casting surface which phase does not transform before the strip has left the casting surface.

The method of the present invention may be carried out in a twin roll caster.

The invention further provides an apparatus for continuously casting metal strip comprising a casting roll having a casting surface to contact a casting pool of molten metal and means to cool the casting surface of the casting roll to cause metal to solidify thereon, the roll surface being formed by a solid coating on a heat conductive roll body, characterised in that the coating is comprised of a substantially amorphous alloy of two components so selected that the wetting angle of the molten metal on the coating surface is less than 40° and the temperature of the coating during metal solidification remains below the melting temperature of the coating.

### BRIEF DESCRIPTION OF THE DRAWINGS

In order that the invention may be more fully explained the results of experimental work carried out to date will be described with reference to the accompanying drawings in which:
Figure 1 illustrates experimental apparatus for determining metal solidification rates under conditions simulating those of a twin roll caster;
Figure 2 illustrates an immersion paddle incorporated in the experimental apparatus of Figure 1;
Figure 3 illustrates thermal resistance values obtained during solidification of a typical steel sample in the experimental apparatus;
Figure 4 illustrates the relationship between wettability of an interface layer and measured heat flux and interface resistance;
Figures 5 illustrates the effect of wettability on the resistance to nucleation;
Figure 6 illustrates shell surface temperatures occurring in steel shells deposited on chromium substrates;
Figure 7 plots the results of heat flux measurements on steel shells deposited on nickel-phosphorus substrate and on chromium substrates;
Figure 8 plots K-value measurements on steel shells deposited during dip tests using nickel-phosphorus alloy and chromium substrates;
Figures 9 and 10 are photomicrographs of steel shells deposited in the dip tests to which Figure 8 refers;
Figure 11, plots K-valve measurements on steel shells deposited during further dip tests using various substrates and steel melt compositions;
Figure 12 to 16 are photomicrographs of steel shells deposited during the dip test to which Figure 11 refers;
Figure 17 is a plan view of a continuous strip caster which is operable in accordance with the invention;
Figure 18 is a side elevation of the strip caster shown in Figure 17;
Figure 19 is a vertical cross-section on the line 19-19 in Figure 17;
Figure 20 is a vertical cross-section on the line 20-20 in Figure 17; and
Figure 21 is a vertical cross-section on the line 21-21 in Figure 17.

### DETAILED DESCRIPTION OF THE PREFERRED EMBODTMENT

Figures 1 and 2 illustrate a metal solidification test rig in which a 40 mm x 40 mm chilled block is advanced into a bath of molten steel at such a speed as to closely simulate the conditions at the casting surfaces of a twin roll caster. Steel solidifies onto the chilled block as it moves through the molten bath to produce a layer of solidified steel on the surface of the block. The thickness of this layer can be measured at points throughout its area to map variations in the solidification rate and therefore the effective rate of heat transfer at the various locations. It is thus possible to produce an overall solidification rate as well as total heat flux measurements. It is also possible to examine the microstructure of the strip surface to correlate changes in the solidification microstructure with the changes in observed solidification rates and heat transfer values.

The experimental rig illustrated in Figures 1 and 2 comprises an induction furnace 1 containing a melt of molten metal 2 in an inert atmosphere which may for example be provided by argon or nitrogen gas. An immersion paddle denoted generally as 3 is mounted on a slider 4 which can be advanced into the melt 2 at a chosen speed and subsequently retracted by the operation of computer controlled motors 5.

Immersion paddle 3 comprises a steel body 6 which contains a substrate 7 in the form of a chrome plated copper disc of 46 mm diameter and 18 mm thickness. It is instrumented with thermo-couples to monitor the temperature rise in the substrate which provides a measure of the heat flux.

Tests carried out on the experimental rig illustrated in Figures 1 and 2 have demonstrated that the observed solidification rates and heat flux values as well as the microstructure of the solidified shell are greatly affected by the conditions at the shell/substrate interface during solidification. The tests have shown that high heat flux and solidification rates can be achieved with smooth substrate surfaces and this can generate refined grain structure of the solidified metal.

During solidification the total resistance to heat flow from the melt to the substrate (heat sink) is governed by the thermal resistances of the solidifying shell and the shell/substrate interface. Under the conditions of conventional continuously cast sections (slabs, blooms or billets), where solidification is completed in around 30 minutes, the heat transfer resistance is dominated by the solidifying shell resistance. However, our experimental work has demonstrated that under thin strip casting conditions, where solidification is completed in less than a second, the heat transfer resistance is dominated by the interface thermal resistance at the surface of the substrate.

The heat transfer resistance is defined as${\text{R}}_{\text{(t)}} {\text{= ΔT}}_{\text{(t)}} {}_{\text{/}} {\text{ΔQ}}_{\text{(t)}}$ where *Q, ΔT* and *t* are heat flux, temperature difference between melt and substrate and time, respectively.

Figure 3 illustrates thermal resistance values obtained during solidification of a typical manganese killed low carbon steel sample in the test rig. This shows that the shell thermal resistance contributes only a small proportion of the total thermal resistance which is dominated by the interface thermal resistance. The interface resistance is initially determined by the melt/substrate interface resistance and later by the shell/substrate interface thermal resistance. Furthermore, it can be seen that the interface thermal resistance does not significantly change in time which indicates that it will be governed by the melt/substrate thermal resistance at the initial melt/substrate contact.

For a two-component system (melt and substrate), the melt/substrate interface resistance and heat flux are determined by the wettability of the melt on a particular substrate. This is illustrated in Figure 4 which shows how interface resistance increases and heat flux decreases with increasing wetting angle which corresponds with reducing wettability.

The importance of wetting of the substrate by the melt was demonstrated by the developmental work described in our aforesaid United States Patent 5,520,243 (International Patent Application PCT/AU93/00593) which discloses application of vibratory movements. The application of vibratory movements was for the purpose of promoting wetting of the substrate and increasing the nucleation density for the melt solidification. The mathematical model described at page 10 of that case proceeded on the basis that full wetting was required and considered the vibrational energy required to achieve this. In the experimental work which verified this analysis it was shown that significant improvement in heat flux could not be obtained unless the substrate was smooth. More specifically, it is necessary for the substrate to have an Arithmetic Mean Roughness Value (Rₐ) of less than 5 microns in order to obtain full wetting of the substrate, even with the application of vibration energy. These results are appropriate for substrates of chromium on which steel melts have moderately good wettability. However, by the present invention the casting surfaces of the rolls can be formed of a material which has a much higher affinity for steel melts so producing much better wetting than can be achieved with a chrome surface. In these circumstances the smoothness of the substrate is not particularly critical although it is desirable in practice that the casting surfaces have an Arithmetic Mean Roughness Value (Rₐ) of less than 10 microns in order to produce strip having a reasonably good surface finish and a refined microstructure.

For metal solidification onto a smooth substrate it can be assumed that solidification will proceed at heterogeneous nucleation sites throughout the substrate. The effect of wetting angle on dimensionless free energy of nucleation according to such classical heterogeneous nucleation theory is illustrated in Figure 5 which shows the manner in which the dimensionless free energy barrier factor increases with increasing wetting angle ie with reducing wetting effectiveness. Wetting angles of 40° and less represent very good wetting effectiveness at which there is a negligible energy barrier to solidification. Wetting angles above 75° represent poor wetting above which there will be a significant energy barrier to metal solidification.

Twin roll strip casters for casting ferrous metals have traditionally employed casting rolls with chromium or nickel casting surfaces generally produced by plating. Such surfaces are tough and are generally able to withstand the thermal stresses associated with strip casting. Moreover, steel melts have moderately good wettability on chromium and nickel surfaces enabling effective heat flux values to be achieved. We have also determined that the metal oxides deposited from typical steel melts used for strip casting have a high affinity for chromium and nickel and they therefore exhibit good wettability on such casting surfaces ie very low wetting angles. This means that there is a very strong tendency for an oxide coating to spread over the casting surfaces and to build up as casting proceeds.

Figure 6 illustrates the measurement of shell surface temperatures occurring in steel shells deposited on chromium surfaces in the dip tested illustrated in Figures 1 and 2 for both a clean substrate surface and a surface with a heavy oxide deposit. It will be seen that for smooth substrate surface the surface of the solidifying shell decreases smoothly in temperature as solidification progresses. Where the substrate has a heavy oxide covering the shell initially proceeds with under-cooling down to a temperature approaching 1200°C at which stage there is a sudden reversal and the temperature of the shell increases. It is thought that the under-cooling proceeds while the oxides are in liquid form but as the temperature approaches 1200°C the oxides solidify to provide nucleation sites for metal solidification. However, the solid oxides then provide a barrier to heat flux with consequent loss of cooling effectiveness and the surface temperature of the shell increases. Previously it was thought that this effect could only be overcome by careful cleaning of the rolls during casting to maintain the oxide levels within a very strict range. However, we have now determined that by forming the casting surfaces from an alternative material which causes extremely good wetting by the steel melt it is possible to cause the steel melt to solidify without significant under-cooling below the liquidus temperature. Such cooling may proceed so rapidly that there is no time for oxidation products to form on the casting surfaces so that solidification proceeds without any significant interference by deposited oxidation products. Specifically these results have been demonstrated by dip testing in the apparatus as illustrated in Figures 1 and 2 using cooling substrates of a nickel-phosphorus alloy comprising 10% phosphorus. This alloy can be coated onto a cooling roll by an electroless process and it promotes very good wetting by steel melts. For most steel melts the wetting angle on this coating would be of the order of 25° or less.

Figure 7 plots heat flux measurements obtained on solidification of a carbon steel onto substrates of the nickel-phosphorus alloy compared with heat flux measurements on solidification of shells of the same steel onto chrome substrates. The carbon steel in these tests had the following composition which we designate an MO6 steel:

| | |
|---|---|
| Carbon | 0.06% by weight |
| Manganese | 0.6% by weight |
| Silicon | 0.28% by weight |
| Aluminium | ≤ 0 . 002% by weight |
| Melt free oxygen | 60-100 parts per million. |

Figure 8 provides the results of measurements of K-value (an indication of heat flux) for multiple dip tests using a carbon steel melt of the above composition and with the nickel-phosphorus alloy and chromium substrates. It will be seen that the results in both Figures 7 and 8 demonstrate that the nickel-phosphorus alloy substrates resulted in much higher heat flux than the normal chrome substrates. In the case of the nickel-phosphorus alloy substrate there was a variation in heat flux over different tests and particularly a decreasing K-value throughout successive dip tests in the results shown in Figure 8. These variations were due to melting of the nickel-phosphorus alloy substrate surface as testing proceeded. Accordingly in order to achieve a long-life coating in a commercial strip caster for casting steel strip at high melt temperatures it would be desirable to modify this particular alloy composition in order to increase its melting temperature. However, the tests demonstrate the dramatically improved results which can be achieved with low wetting angles and the nickel-phosphorus alloy as tested would be entirely suitable for use in casting of other metals such as copper.

Figures 9 and 10 are photomicrographs of MO6 steel shells deposited onto substrates of nickel-phosphorus alloy in the case of Figure 9 and a traditionally chromium substrate in the case of Figure 10, both photomicrographs being shown to a magnification of x100. It will be seen that the shell deposited onto the nickel-phosphorus alloy substrate is almost twice as thick as the shell deposited on the chromium substrate, reflecting the much higher heat flux and more rapid solidification obtained with the nickel-phosphorus alloy substrate. This demonstrates that very much higher solidification rates are achievable and that accordingly the invention will permit strip casting to proceed at dramatically higher production rates than have hitherto been thought possible. Moreover, it will be seen that the microstructure of the shell deposited on the nickel-phosphorus alloy substrate is significantly finer than that deposited on the traditional chrome substrate and is moreover remarkably even throughout the shell. This microstructure exhibits prior austenite grain boundaries that exactly follow dendritic grain boundaries demonstrating that the liquid carbon steel has solidified directly into austenite. With this solidification process there is no potential for the development of crocodile-skin defects since these defects arise only when both δ and γ phases are present in the solidifying steel shells.

It has been found that the enhanced wettability of the nickel-phosphorus alloy is due to its amorphous structure. Liquids will in general have a high surface affinity for other liquids since they have no preferential orientation and we have now found that a similar effect can be produced when wetting an amorphous solid. Wettability of a liquid metal on a coating surface can accordingly be dramatically increased if the coating material is totally amorphous. The nickel-phosphorus alloy with a 10% phosphorus content, as used in the tests to which Figures 8 and 9 refer, is a substantially eutectic composition and can readily be deposited by an electroless process so as to have an effectively totally amorphous structure. If the phosphorus content is varied so as to depart significantly from the eutectic composition the deposited nickel-phosphorus alloy coating will exhibit a partially crystalline structure rather than being totally amorphous. Moreover, a crystalline structure can also be produced by annealing the coating at elevated temperature after deposition, a phenomenon that is used to increase hardness in some coating applications.

In order to demonstrate the effect of an amorphous coating in enhancing wettability and heat flux in accordance with the invention, we have conducted a series of further tests in which steel melts have been solidified on nickel-phosphorus alloy substrates of varying phosphorus composition, on nickel-phosphorus alloy substrates which were annealed at elevated temperature prior to testing and also on smooth nickel substrates to provide standard or control data. Moreover, in order to further demonstrate the direct solidification of steel directly into austenite dendrites in accordance with the invention the further tests included the deposition of shells from a peritectic grade steel which would normally produce gross distortions on solidification through solidification into δ and γ phases simultaneously. The results of this further testing are illustrated by Figures 11 to 16.

Figure 11 provides the results of measurements of K-value for multiple dip tests. Dip tests 1-27 all used steel melts having the above described MO6 composition. In tests 1-9 steel shells were deposited on both a smooth nickel substrate having an Rₐ value of 5.6 and on a nickel-phosphorus alloy substrate having a 10% phosphorus content and a Mean Roughness Value (Rₐ) of 8.7.

The nickel-phosphorus substrate used in tests 1-9 was deposited by an electroless process and was not annealed. It will be seen that very high K-values were achieved with this substrate as compared with the smooth nickel substrate used as a control. These results are quite similar to those shown in Figure 8.

Figure 8 further shows results of tests 10-15 in which the nickel substrate was maintained as a control comparison against results for solidification onto a nickel-phosphorus alloy substrate having a phosphorus content of 5% and an Arithmetic Mean Roughness Value (Rₐ) of 6.6. It will be seen that the K-value achieved with the 5% phosphorus alloy was significantly less than that with the 10% phosphorus alloy of tests 1-9, even though a smoother substrate was employed, demonstrating that the partially crystalline structure inevitable in the 5% phosphorus alloy has reduced wetting and total heat flux.

Figure 11 further shows the results of tests 16-23 in which MO6 steel shells were deposited on smooth nickel-phosphorus alloy substrates which all had a 10% phosphorus content but in which one of the substrates had been subjected to annealing at 400°C for 1.5 hours after electroless deposition and the other substrate was not subjected to any annealing. It will be seen that the substrate not subjected to annealing produced the high K-values as previously experienced in tests 1-9 whereas the annealed substrate produced much lower K-values comparable with those achieved with the plain nickel substrate. Figure 12 is a photomicrograph of the shell deposited on the nickel substrate in test number 11, Figure 13 is a photomicrograph of the shell deposited on the annealed substrate in dip test number 18 and Figure 14 is a photomicrograph of the shell deposited on the unannealed nickel-phosphorus alloy substrate in the same dip test number 18. It will be seen that the microstructures exhibited in the shells deposited on the nickel substrate in test 11 and the annealed substrate in test 18 are similar. In both cases the shells are relatively thin and have coarse microstructure exhibiting initial solidification into ferrite. The shell of Figure 14 as deposited onto the unannealed alloy substrate is very much thicker and exhibits the finer microstructure associated with the extremely high solidification rates achievable in accordance with the present invention which result in initial solidification directly into austenite.

Figure 8 further provides the results of tests 24-27 in which shells were deposited on a nickel-phosphorus alloy substrate having a 10% phosphorus content but only partially annealed at 400°C for 45 minutes as compared with a control substrate of nickel as previously used in tests 1-15. It will be seen that the partially annealed substrate resulted in K-values generally between those of the unannealed and annealed substrates of tests 16-23, further demonstrating the effect of an amorphous coating and the graded reduction of K-value and heat flux according to the degree to which a crystalline structure is present in the coating.

Figure 11 also provides results obtained from tests 29-31 in which shells were deposited on a nickel-phosphorus alloy substrate of 10% phosphorus content from a peritectic steel composition having a carbon content of 0.13%. Normally a steel of such composition cannot be cast with good surface quality by direct thin strip casting techniques because the steel solidifies simultaneously into δ and γ ferrite phases and produces gross distortions in the solidifying shell. In the present tests however, the peritectic steel composition produced a shell demonstrating the same microstructure as previously achieved with MO6 steels on the nickel-phosphorus alloy substrates and with the same K-values, demonstrating a similar heat flux on solidif ication.

The solidification structure of the shell of peritectic steel produced in test number 30 is shown in Figure 15 and the solidification structure of a shell of the same steel deposited onto a textured chrome substrate is shown in Figure 16. It will be seen that the structure of Figure 15 is much the same as that exhibited in Figures 9 and 14 and exhibits prior austenite grain boundaries demonstrating that the liquid carbon steel has solidified directly into austenite. Moreover, there is no indication of any ferrite growth even after solidification has progressed to the stage where the cooling rate has decreased. This indicates that when austenitic solidification is initiated in accordance with the invention in a strip casting process there will be a complete transformation into austenite without any reversion to ferrite growth, although there will of course be a subsequent transformation at lower temperatures after the strip has left the casting surface or surfaces.

In the practice of the invention the material of the casting surfaces of the rolls must have a melting temperature higher than the temperature of the casting surfaces during metal solidification. The temperature of the casting surfaces will be dependent on the wetting angle of the molten metal on the casting surfaces. More specifically, the temperature that the casting surface coating experiences will be higher as the wetting angle decreases. The coating material may therefore be chosen so as to provide a balance between high heat flux and rapid solidification and maintenance of a coating temperature which is safely below the melting temperature of the coating.

The results illustrated in Figures 8 and 11 for the unannealed nickel-phosphorus substrates show a progressive loss of performance due to erosion of the coating. For high temperature steel casting, other two metal amorphous coatings may be used in accordance with the invention. For selection of suitable coating it is necessary to take into account the melting temperature of the coating, the interface temperature during casting and the annealing temperature of the coating. Table 1 sets out the relevant criteria for a number of possible alloy coatings which might be used in accordance with the invention in the casting of thin strip steel.

**Table 1**

| Coating | Tinterface (C) | T melt (C) | T crystal (C) | Method of deposition |
|---|---|---|---|---|
| Ni-P | 750 | 870 | 200 | Electroless |
| Ni-B | 750 | 1065 (1018) | -- | Electroless/thermal spray |
| Mo-P | 730 | 1650 | 431 | Electroless |
| Mo-B | 730 | 2180 | -- | PVD / CVD |
| Cr-B | 780 | 1630 | -- | PVD / thermal spray / CVD |
| Ti-P | 1082 | 1495 | 882 | -- |
| Ti-B | 1082 | 1540 | 884 | PVD / CVD |
| Ta-B | 882 | 2390 | 2050? | PVD / CVD |
| W-B | 707 | 1970 | -- | PVD / CVD |
| Co-P | 843 | 1023 | -- | -- |
| Co-B | 843 | 1110 | -- | -- |
| Zr-B | | 1680 | 863 | PVD / thermal spray / CVD |
| Fe-P | 983 | 1048 | 735 | -- |
| Fe-B | 983 | 1174 | 912 | CVD |
| V-B | 980 | 1735 | -- | CVD |

In table 1, the interface temperature has been calculated on the assumption of perfect contact of a steel metal at 1650°C with a coating of 25°C.

Figures 17 to 21 illustrate a twin roll continuous strip caster which may be operated in accordance with the present invention. This caster comprises a main machine frame 11 which stands up from the factory floor 12. Frame 11 supports a casting roll carriage 13 which is horizontally movable between an assembly station 14 and a casting station 15. Carriage 13 carries a pair of parallel casting rolls 16 to which molten metal is supplied during a casting operation from a ladle 17 via a tundish 18 and delivery nozzle 19 to create a casting pool 30. Casting rolls 16 are water cooled so that shells solidify on the moving roll surfaces 16A and are brought together at the nip between them to produce a solidified strip product 20 at the roll outlet. This product is fed to a standard coiler 21 and may subsequently be transferred to a second coiler 22. A receptacle 23 is mounted on the machine frame adjacent the casting station and molten metal can be diverted into this receptacle via an overflow spout 24 on the tundish or by withdrawal of an emergency plug 25 at one side of the tundish if there is a severe malformation of product or other severe malfunction during a casting operation.

Roll carriage 13 comprises a carriage frame 31 mounted by wheels 32 on rails 33 extending along part of the main machine frame 11 whereby roll carriage 13 as a whole is mounted for movement along the rails 33. Carriage frame 31 carries a pair of roll cradles 34 in which the rolls 16 are rotatably mounted. Roll cradles 34 are mounted on the carriage frame 31 by interengaging complementary slide members 35, 36 to allow the cradles to be moved on the carriage under the influence of hydraulic cylinder units 37, 38 to adjust the nip between the casting rolls 16 and to enable the rolls to be rapidly moved apart for a short time interval when it is required to form a transverse line of weakness across the strip as will be explained in more detail below. The carriage is movable as a whole along the rails 33 by actuation of a double acting hydraulic piston and cylinder unit 39, connected between a drive bracket 40 on the roll carriage and the main machine frame so as to be actuable to move the roll carriage between the assembly station 14 and casting station 15 and vice versa.

Casting rolls 16 are contra rotated through drive shafts 41 from an electric motor and transmission mounted on carriage frame 31. Rolls 16 have copper peripheral walls formed with a series of longitudinally extending and circumferentially spaced water cooling passages supplied with cooling water through the roll ends from water supply ducts in the roll drive shafts 41 which are connected to water supply hoses 42 through rotary glands 43. The roll may typically be about 500 mm diameter and up to 2000 mm long in order to produce 2000 mm wide strip product.

Ladle 17 is of entirely conventional construction and is supported via a yoke 45 on an overhead crane whence it can be brought into position from a hot metal receiving station. The ladle is fitted with a stopper rod 46 actuable by a servo cylinder to allow molten metal to flow from the ladle through an outlet nozzle 47 and refractory shroud 48 into tundish 18.

Tundish 18 is also of conventional construction. It is formed as a wide dish made of a refractory material such as magnesium oxide (MgO). One side of the tundish receives molten metal from the ladle and is provided with the aforesaid overflow 24 and emergency plug 25. The other side of the tundish is provided with a series of longitudinally spaced metal outlet openings 52. The lower part of the tundish carries mounting brackets 53 for mounting the tundish onto the roll carriage frame 31 and provided with apertures to receive indexing pegs 54 on the carriage frame so as to accurately locate the tundish.

Delivery nozzle 19 is formed as an elongate body made of a refractory material such as alumina graphite. Its lower part is tapered so as to converge inwardly and downwardly so that it can project into the nip between casting rolls 16. It is provided with a mounting bracket 60 whereby to support it on the roll carriage frame and its upper part is formed with outwardly projecting side flanges 55 which locate on the mounting bracket.

Nozzle 19 may have a series of horizontally spaced generally vertically extending flow passages to produce a suitably low velocity discharge of metal throughout the width of the rolls and to deliver the molten metal into the nip between the rolls without direct impingement on the roll surfaces at which initial solidification occurs. Alternatively, the nozzle may have a single continuous slot outlet to deliver a low velocity curtain of molten metal directly into the nip between the rolls and/or it may be immersed in the molten metal pool.

The pool is confined at the ends of the rolls by a pair of side closure plates 56 which are held against stepped ends 57 of the rolls when the roll carriage is at the casting station. Side closure plates 56 are made of a strong refractory material, for example boron nitride, and have scalloped side edges 81 to match the curvature of the stepped ends 57 of the rolls. The side plates can be mounted in plate holders 82 which are movable at the casting station by actuation of a pair of hydraulic cylinder units 83 to bring the side plates into engagement with the stepped ends of the casting rolls to form end closures for the molten pool of metal formed on the casting rolls during a casting operation.

During a casting operation the ladle stopper rod 46 is actuated to allow molten metal to pour from the ladle to the tundish through the metal delivery nozzle whence it flows to the casting rolls. The clean head end of the strip product 20 is guided by actuation of an apron table 96 to the jaws of the coiler 21. Apron table 96 hangs from pivot mountings 97 on the main frame and can be swung toward the coiler by actuation of an hydraulic cylinder unit 98 after the clean head end has been formed. Table 96 may operate against an upper strip guide flap 99 actuated by a piston and a cylinder unit 101 and the strip product 20 may be confined between a pair of vertical side rollers 102. After the head end has been guided in to the jaws of the coiler, the coiler is rotated to coil the strip product 20 and the apron table is allowed to swing back to its inoperative position where it simply hangs from the machine frame clear of the product which is taken directly onto the coiler 21. The resulting strip product 20 may be subsequently transferred to coiler 22 to produce a final coil for transport away from the caster.

Full particulars of a twin roll caster of the kind illustrated in Figures 11 to 15 are more fully described in our United States Patents 5,184,668 and 5,277,243 and International Patent Application PCT/AU93/00593.

## Claims

1. A method for continuously casting metal strip of the kind in which a casting pool of molten metal is formed in contact with a moving casting surface such that metal solidifies from the pool onto the moving casting surface, wherein the casting surface is provided by a solid coating on a heat conductive body, **characterised in that** the coating material is so selected that the wetting angle of said molten metal. on the coating surface is less than 40°, and the temperature of the coating during metal solidification is maintained below the melting temperature of the coating.

2. A method as claimed in claim 1, wherein the coating is formed of a material such that the wetting angle of the molten metal on the coating surface is less than 20°.

3. A method as claimed in claim 1 or claim 2, wherein the coating surface has an Arithmetic Mean Roughness Value (Rₐ) of less than 10 microns.

4. A method as claimed in any one of the preceding claims, wherein the molten metal is molten steel.

5. A method as claimed in claim 4, wherein the steel solidifies into a single phase solid structure on the casting surface.

6. A method as claimed in any one of the preceding claims, wherein the coating material is at least partially amorphous.

7. A method as claims in claim 6, wherein the coating material is substantially totally amorphous.

8. A method as claimed in any one of the preceding claims, wherein the coating material is comprised of an alloy of two components .

9. A method as claimed in claim 8, wherein one of the components of the alloy is phosphorus.

10. A method as claimed in claim 9, wherein the other component of the said alloy is nickel.

11. A method as claimed in any one of claims 8 to 10, wherein said alloy is a substantially eutectic alloy.

12. A method as claimed in any one of the preceding claims, wherein the molten metal has a substantially eutectic composition.

13. A method as claimed in any one of the preceding claims, wherein the heat conductive body is a copper or copper alloy body.

14. A method for continuously casting steel strip of the kind in which a casting pool of molten steel is formed in contact with a moving casting surface such that steel solidifies from the casting pool onto the moving casting surface, wherein the casting surface is provided by a solid coating on a heat conductive body, **characterised in that** the coating material is so selected that the wetting angle of the molten metal on the coating surface is less than 40°, the temperature of the coating during metal solidification is maintained below the melting temperature of the coating, and wherein the steel solidifies into a single phase solid structure on the casting surface which phase does not transform before the strip has left the casting surface.

15. A method as claimed in claim 14, wherein said steel has a carbon equivalent content of not more than 0.13% by weight and said single phase structure comprises dendrites of solid austenite.

16. A method as claimed in claim 15, wherein the steel has a substantially peritectic composition.

17. A method as claimed in claim 16, wherein the steel has a carbon content of about 0.13% by weight.

18. A method as claimed in any one of claims 14 to 17, wherein the coating material is comprised of an amorphous alloy of two components.

19. A method as claimed in claim 18, wherein one of the components of the alloy is phosphorus.

20. A method as claimed in claim 19, wherein the coating is a nickel-phosphorus alloy containing about 10% phosphorus.

21. A method as claimed in any one of claims 14 to 20, wherein the heat conductive body is a copper or copper alloy body.

22. A method as claimed in any one of claims 14 to 21, wherein the moving casting surface is one of a pair of such surfaces being the surfaces of a pair of casting rolls forming a nip between them, the casting pool being supported on the casting rolls above the nip and the strip being delivered downwardly from the nip with said single phase solid structure.

23. A method for continuously casting metal strip of the kind in which a casting pool of molten metal is formed in contact with a moving casting surface such that metal solidifies from the casting pool onto the moving casting surface, wherein the metal is of peritectic composition, the casting surface is provided by a solid coating on a heat conductive body, **characterised in that** the coating material is so selected that the wetting angle of the molten metal on the coating surface is less than 40°, the temperature of the coating during metal solidification is maintained below the melting temperature of the coating, and wherein the metal solidifies into a single phase solid structure on the casting surface which phase does not transform before the strip has left the casting surface.

24. Apparatus for continuously casting metal strip comprising a casting roll having a casting surface to contact a casting pool of molten metal and means to cool the casting surface of the casting roll to cause metal to solidify thereon, the roll surface being formed by a solid coating on a heat conductive body of the roll, **characterised in that** the coating is comprised of a substantially amorphous alloy of two components so selected that the wetting angle of the molten metal on the coating surface is less than 40° and the temperature of the coating during metal solidification remains below the melting temperature of the coating.

25. Apparatus as claimed in claim 24, wherein one of the components of the alloy is phosphorus.

26. Apparatus as claimed in claim 25, wherein the coating alloy is a nickel-phosphorus alloy.

27. Apparatus as claimed in claim 26, wherein the coating alloy contains about 10% phosphorus.

28. A casting roll comprising a heat conductive cylindrical roll body covered by a solid coating defining a cylindrical metal casting surface, **characterised in that** the coating is comprised of a substantially amorphous alloy of two components.

29. A casting roll as claimed in claim 28, wherein one of the components of the alloy is phosphorus.

30. A casting roll as claimed in claim 29, wherein the coating alloy is a nickel-phosphorus alloy.

31. A casting roll as claimed in claim 30, wherein the coating alloy contains about 10% phosphorus.

## Patentansprüche

1. Verfahren zum Stranggießen von Metallband des Typs, bei dem ein Gießsumpf aus geschmolzenem Metall in Kontakt mit einer sich bewegenden Gießfläche ausgebildet wird, so dass sich das Metall aus dem Sumpf heraus auf der sich bewegenden Gießfläche verfestigt, wobei die Gießfläche durch eine feste Beschichtung auf einem wärmeleitenden Körper gebildet wird, **dadurch gekennzeichnet, dass** das Beschichtungsmaterial so ausgewählt wird, dass der Benetzungswinkel des geschmolzenen Metalls auf der Beschichtungsfläche weniger als 40° beträgt und die Temperatur der Beschichtung während der Metallverfestigung unter der Schmelztemperatur der Beschichtung gehalten wird.

2. Verfahren nach Anspruch 1, wobei die Beschichtung aus einem Material ausgebildet ist, durch das der Benetzungswinkel des geschmolzenen Metalls auf der Beschichtungsfläche weniger als 20° beträgt.

3. Verfahren nach Anspruch 1 oder Anspruch 2, wobei die Beschichtungsfläche ein Mittenrauwert (Rₐ) von weniger als 10 Mikrometer hat.

4. Verfahren nach einem der vorangehenden Ansprüche, wobei das geschmolzene Metall geschmolzener Stahl ist.

5. Verfahren nach Anspruch 4, wobei sich der Stahl zu einer einphasigen festen Struktur auf der Gießfläche verfestigt.

6. Verfahren nach einem der vorangehenden Ansprüche, wobei das Beschichtungsmaterial wenigstens teilweise amorph ist.

7. Verfahren nach Anspruch 7, wobei das Beschichtungsmaterial im Wesentlichen vollkommen amorph ist.

8. Verfahren nach einem der vorangehenden Ansprüche, wobei das Beschichtungsmaterial aus einer Legierung aus zwei Komponenten besteht.

9. Verfahren nach Anspruch 8, wobei eine der Komponenten der Legierung Phosphor ist.

10. Verfahren nach Anspruch 9, wobei die andere Komponente der Legierung Nickel ist.

11. Verfahren nach einem der Ansprüche 8 bis 10, wobei die Legierung eine im Wesentlichen eutektische Legierung ist.

12. Verfahren nach einem der vorangehenden Ansprüche, wobei das geschmolzene Metall eine im Wesentlichen eutektische Zusammensetzung hat.

13. Verfahren nach einem der vorangehenden Ansprüche, wobei der wärmeleitende Körper ein Kupfer- oder Kupferlegierungskörper ist.

14. Verfahren zum Stranggießen von Stahlband des Typs, bei dem ein Gießsumpf aus geschmolzenem Stahl in Kontakt mit einer sich bewegenden Gießfläche so ausgebildet wird, dass sich der Stahl aus dem Gießsumpf heraus auf der sich bewegenden Gießfläche verfestigt, wobei die-Gießfläche durch eine feste Beschichtung auf einem wärmeleitenden Körper gebildet wird, **dadurch gekennzeichnet, dass** das Beschichtungsmaterial so ausgewählt wird, dass der Benetzungswinkel des geschmolzenen Metalls auf der Beschichtungsfläche weniger als 40° beträgt, wobei die Temperatur der Beschichtung während der Metallverfestigung unter der Schmelztemperatur der Beschichtung gehalten wird, und wobei sich der Stahl zu einer einphasigen festen Struktur auf der Gießfläche verfestigt und sich die Phase nicht umwandelt, bevor das Band die Gießfläche verlassen hat.

15. Verfahren nach Anspruch 14, wobei der Stahl einen Kohlenstoff-Äquivalentgehalt von nicht mehr als 0,13 Gew.-% hat und die einphasige Struktur Dendrite aus festem Austenit umfasst.

16. Verfahren nach Anspruch 15, wobei der Stahl eine im Wesentlichen peritektische Zusammensetzung hat.

17. Verfahren nach Anspruch 16, wobei der Stahl einen Kohlenstoffgehalt von ungefähr 0,13 Gew.-% hat.

18. Verfahren nach einem der Ansprüche 14 bis 17, wobei das Beschichtungsmaterial aus einer amorphen Legierung aus zwei Komponenten besteht.

19. Verfahren nach Anspruch 18, wobei eine der Komponenten der Legierung Phosphor ist.

20. Verfahren nach Anspruch 19, wobei die Beschichtung eine Nickel-Phosphor-Legierung ist, die ungefähr 10% Phosphor enthält.

21. Verfahren nach einem der Ansprüche 14 bis 20, wobei der wärmeleitende Körper ein Kupfer- oder Kupferlegierungskörper ist.

22. Verfahren nach einem der Ansprüche 14 bis 21, wobei die sich bewegende Gießfläche eine eines Paars derartiger Flächen ist, die die Flächen eines Paars Gießwalzen sind, die einen Spalt zwischen einander bilden, wobei der Gießsumpf auf den Gießwalzen über dem Spalt getragen wird und das Band aus dem Spalt mit der einphasigen festen Struktur nach unten ausgegeben wird.

23. Verfahren zum Stranggießen von Metallband des Typs, bei dem ein Gießsumpf aus geschmolzenem Metall in Kontakt mit einer sich bewegenden Gießfläche so ausgebildet wird, dass sich das Metall aus dem Gießsumpf heraus auf der sich bewegenden Gießfläche verfestigt, wobei das Metall peritektische Zusammensetzung hat, die Gießfläche durch eine feste Beschichtung auf einem wärmeleitenden Körper gebildet wird, **dadurch gekennzeichnet, dass** das Beschichtungsmaterial so ausgewählt wird, dass der Benetzungswinkel des geschmolzenen Materials auf der Beschichtungsfläche weniger als 40° beträgt, wobei die Temperatur der Beschichtung während der Metallverfestigung unter der Schmelztemperatur der Beschichtung gehalten wird, und wobei sich das Metall zu einer einphasigen festen Struktur auf der Gießfläche verfestigt und diese Phase sich nicht umwandelt, bevor das Band die Gießfläche verlassen hat.

24. Vorrichtung zum Stranggießen von Metallband, die eine Gießwalze mit einer Gießfläche, die mit einem Gießsumpf aus geschmolzenem Metall in Kontakt kommt, und eine Einrichtung, die die Gießfläche der Gießwalze abkühlt, um zu bewirken, dass sich Metall darauf verfestigt, wobei die Walzenoberfläche durch eine feste Beschichtung auf einem wärmeleitenden Körper der Walze gebildet wird, **dadurch gekennzeichnet, dass** die Beschichtung aus einer im Wesentlichen amorphen Legierung aus zwei Komponenten besteht, die so ausgewählt werden, dass der Benetzungswinkel des geschmolzenen Metalls auf der Beschichtungsfläche weniger als 40° beträgt und die Temperatur der Beschichtung während der Metallverfestigung unter der Schmelztemperatur der Beschichtung bleibt.

25. Vorrichtung nach Anspruch 24, wobei eine der Komponenten der Legierung Phosphor ist.

26. Vorrichtung nach Anspruch 25, wobei die Beschichtungslegierung eine Nickel-Phosphor-Legierung ist.

27. Vorrichtung nach Anspruch 26, wobei die Beschichtungslegierung ungefähr 10% Phosphor enthält.

28. Gießwalze, die einen wärmeleitenden zylindrischen Walzenkörper umfasst, der mit einer festen Beschichtung überzogen ist, die eine zylindrische Metallgießfläche bildet, **dadurch gekennzeichnet, dass** die Beschichtung aus einer im Wesentlichen amorphen Legierung aus zwei Komponenten besteht.

29. Gießwalze nach Anspruch 28, wobei eine der Komponenten der Legierung Phosphor ist.

30. Gießwalze nach Anspruch 29, wobei die Beschichtungslegierung eine Nickel-Phosphor-Legierung ist.

31. Gießwalze nach Anspruch 30, wobei die Beschichtungslegierung ungefähr 10% Phosphor enthält.

## Revendications

1. Procédé pour la coulée continue de bande métallique du type dans lequel un bain de métal en fusion se forme au contact d'une surface de coulée mobile, de sorte que le métal se solidifie du bain sur la surface de coulée mobile, dans lequel la surface de coulée est constituée par un revêtement solide sur un corps thermoconducteur, **caractérisé en ce que** le matériau de revêtement est sélectionné de telle sorte que l'angle de mouillage dudit métal en fusion sur la surface de revêtement soit inférieur à 40° et que la température du revêtement pendant la solidification du métal se maintienne au-dessous de la température de fusion du revêtement.

2. Procédé selon la revendication 1, dans lequel le revêtement est formé d'un matériau tel que l'angle de mouillage du métal en fusion sur la surface de revêtement est inférieur à 20°.

3. Procédé selon la revendication 1 ou la revendication 2, dans lequel la surface de revêtement a une rugosité moyenne arithmétique (Ra) de moins de 10 micromètres.

4. Procédé selon l'une quelconque des revendications précédentes, dans lequel le métal en fusion est de l'acier en fusion.

5. Procédé selon la revendication 4, dans lequel l'acier se solidifie en une structure solide monophasique sur la surface de coulée.

6. Procédé selon l'une quelconque des revendications précédentes, dans lequel le matériau de revêtement est au moins partiellement amorphe.

7. Procédé selon la revendication 6, dans lequel le matériau de revêtement est, sensiblement complètement amorphe.

8. Procédé selon l'une quelconque des revendications précédentes, dans lequel le matériau de revêtement est composé d'un alliage de deux composants.

9. Procédé selon la revendication 8, dans lequel l'un des composants de l'alliage est le phosphore.

10. Procédé selon la revendication 9, dans lequel l'autre composant dudit alliage est le nickel.

11. Procédé selon l'une quelconque des revendications 8 à 10, dans lequel ledit alliage est en substance un alliage eutectique.

12. Procédé selon l'une quelconque des revendications précédentes, dans lequel le métal en fusion a une composition sensiblement eutectique.

13. Procédé selon l'une quelconque des revendications précédentes, dans lequel le corps thermoconducteur est un corps en cuivre ou en alliage de cuivre.

14. Procédé pour la coulée continue de bande métallique, du type dans lequel un bain de métal en fusion se forme au contact d'une surface de coulée mobile, de sorte que l'acier se solidifie du bain sur la surface de coulée mobile, dans lequel la surface de coulée est constituée par un revêtement solide sur un corps thermoconducteur, **caractérisé en ce que** le matériau de revêtement est sélectionné de telle sorte que l'angle de mouillage dudit métal en fusion sur la surface de revêtement soit inférieur à 40° et que la température du revêtement pendant la solidification du métal se maintienne au-dessous de la température de fusion du revêtement, et dans lequel l'acier se solidifie en une structure solide monophasique sur la surface de coulée, laquelle phase ne se transforme pas avant que la bande n'ait quitté la surface de coulée.

15. Procédé selon la revendication 14, dans lequel ledit acier a une teneur en carbone équivalent ne dépassant pas 0,13% en poids et ladite structure monophasique comprend des dendrites d'austénite solide.

16. Procédé selon la revendication 15, dans lequel l'acier a une composition sensiblement péritectique.

17. Procédé selon la revendication 16, dans lequel l'acier a une teneur en carbone d'environ 0,13% en poids.

18. Procédé selon l'une quelconque des revendications 14 à 17, dans lequel le matériau de revêtement est composé d'un alliage amorphe de deux composants.

19. Procédé selon la revendication 18, dans lequel l'un des composants de l'alliage est le phosphore.

20. Procédé selon la revendication 19, dans lequel le revêtement est un alliage de nickel-phosphore contenant environ 10% de phosphore.

21. Procédé selon l'une quelconque des revendications 14 à 20, dans lequel le corps thermoconducteur est un corps en cuivre ou en alliage de cuivre.

22. Procédé selon l'une quelconque des revendications 14 à 21, dans lequel la surface de coulée mobile est l'une des surfaces d'une paire de cyclindres de moulage formant un étranglement entre eux, le bain de moulage étant soutenu sur les cylindres de moulage au-dessus de l'étranglement et la bande étant libérée vers le bas à partir de l'étranglement avec ladite structure solide monophasique.

23. Procédé pour la coulée continue de bande métallique, du type dans lequel un bain de métal en fusion se forme au contact d'une surface de coulée mobile, de sorte que le métal se solidifie du bain sur la surface de coulée mobile, dans lequel le métal est de composition péritectique, la surface de coulée est constituée par un revêtement solide sur un corps thermoconducteur, **caractérisé en ce que** le matériau de revêtement est sélectionné de telle sorte que l'angle de mouillage du métal en fusion sur la surface de revêtement soit inférieur à 40° et que la température du revêtement pendant la solidification du métal se maintienne au-dessous de la température de fusion du revêtement, et dans lequel le métal se solidifie en une structure solide monophasique sur la surface de coulée, laquelle phase ne se transforme pas avant que la bande n'ait quitté la surface de coulée.

24. Appareil pour la coulée continue de bande métallique comprenant un cyclindre de coulée ayant une surface de coulée pour entrer au contact d'un bain de métal en fusion et un moyen pour refroidir la surface de coulée du cyclindre de coulée pour faire que le métal se solidifie dessus, la surface du cylindre étant formée par un revêtement solide sur un corps thermoconducteur du cylindre, **caractérisé en ce que** le revêtement est composé d'un alliage sensiblement amorphe de deux composants sélectionnés de telle sorte que l'angle de mouillage du métal en fusion sur la surface de coulée soit inférieur à 40° et que la température du revêtement pendant la solidification du métal reste inférieure à la température de fusion du revêtement.

25. Appareil selon la revendication 24, dans lequel l'un des composants de l'alliage est le phosphore.

26. Appareil selon la revendication 25, dans lequel l'alliage de revêtement est un alliage de nickel-phosphore.

27. Appareil selon la revendication 26, dans lequel l'alliage de revêtement contient environ 10% de phosphore.

28. Cyclindre de coulée composé d'un corps cyclindrique thermoconducteur recouvert d'un revêtement solide, définissant une surface de coulée métallique cylindique, **caractérisé en ce que** le revêtement est composé d'un alliage sensiblement amorphe de deux composants.

29. Cylindre de coulée selon la revendication 28, dans lequel l'un des composants de l'alliage est le phosphore.

30. Cylindre de coulée selon la revendication 29, dans lequel l'alliage de revêtement est un alliage de nickel-phosphore.

31. Cylindre de coulée selon la revendication 30, dans lequel l'alliage de revêtement contient environ 10% de phosphore.
